

## UNITED STATES PATENT OFFICE

GEORGE A. RICHTER, OF BERLIN, NEW HAMPSHIRE, ASSIGNOR TO BROWN COMPANY, OF BERLIN, NEW HAMPSHIRE, A CORPORATION OF MAINE

## MULTIPLE-STEP PROCESS OF FIBER LIBERATION

No Drawing.

Application filed May 6, 1930. Serial No. 450,314.

This invention relates to the liberation of fiber from raw cellulosic materials to produce a pulp which at the time of liberation is practically free from non-alpha cellulose components, including pentosans, and which is characterized by a low so-called solution viscosity, which renders it especially valuable for conversion into derivatives to be treated with solvents to form solutions of low viscosity.

In accordance with the process of the present invention, three chemical liquors of different compositions are employed in the treatment of the cellulosic material before its fiber content is isolated as pulp freed from the associated organic materials. Each liquor exerts a chemical action on the cellulosic material, and thus contributes to the results secured, but there is a preferable sequence in which the liquors are used. The first liquor employed is a sulphurous acid solution which is especially effective for removing pentosans from the raw cellulosic material and in so modifying the constitution of the cellulose fibers as to lead to a final product of low solution viscosity. The second liquor is a bisulphite solution which may be added to the cellulosic material after the sulphurous acid solution has been drained therefrom, or which may be prepared from the sulphurous acid solution by adding suitable chemicals thereto. The bisulphite solution is an active agency in the removal of ligneous matter contained in the cellulosic material and in conditioning the cellulosic material for the treatment with the third chemical liquor, which brings about complete fiber liberation. The third chemical liquor is a solution of alkali, such as that used in the soda or kraft process, which, even at low concentrations, readily completes the removal of residual ligneous matter contained in the cellulosic material to effect complete fiber liberation.

The treatment of the cellulosic material with a bisulphite liquor between the first treatment with a sulphurous acid solution and the treatment with a solution of alkali is advantageous, in that it not only makes possible a reduction in the quantity of alkali

necessary to complete fiber liberation, but also a higher yield of pulp, based on wood, without impairing the bleachability of the pulp. The intermediate treatment with the bisulphite liquor is effected under conditions designed not to isolate the fiber content of the cellulosic material. The combined  $SO_2$  content desired in the bisulphite liquor may be obtained by adding alkali, such as caustic soda, sodium sulphite, or sodium sulphate to the sulphurous acid solution remaining after the first treatment. These chemicals may be added in the form of concentrated solutions in amount calculated to produce the desired combined  $SO_2$  content. When such a procedure is followed, heat consumed in raising the temperature of the sulphurous acid solution of the first treatment is conserved for the second treatment. The sulphur dioxide content of the first treating solution is also conserved for the preparation of the bisulphite solution used in the second treatment; and the time lost when the first treating solution is drained from the chips and replaced by a previously prepared bisulphite solution is avoided.

The process of the present invention is applicable to various raw cellulosic materials which are of high pentosan content as found in material such as hardwoods, hemp, bamboo, and bagasse. It is also applicable to wood such as spruce, which is an excellent raw material for the production of pulps of high alpha cellulose content and suitable both for papermaking and for the preparation of cellulose derivatives. A specific example of procedure which may be practised with eminently successful results in the case of spruce, may be substantially as follows. The chipped wood, which may be in the form of chips of the normal size, or of a size larger or smaller than that usually employed in a pulp mill, is first treated with a sulphurous acid solution containing about 2% to 5%  $SO_2$ . This treatment may be effected in a digester in which the charge of wood and liquor may be confined under pressure and at elevated temperature. The digester contents are heated to a temperature of 230° to 260° F., which is maintained for about two hours while the pressure is ordinarily not allowed to exceed 100

about 60 to 75 pounds; but in special cases higher pressure may be reached. At the end of this time, the solution may be drained from the chips and a suitable bisulphite liquor 5 added to the digester, but it is preferable to form the bisulphite liquor from the sulphurous acid solution of the first treatment. Accordingly, a concentrated solution of caustic soda, sodium sulphite, or sodium sulphate 10 may be added to the sulphurous acid solution until the desired combined  $\text{SO}_2$  content is produced therein, say, 1% to 2%, or greater. When sodium sulphate is the added chemical, only a relatively small portion will react 15 with the sulphurous acid solution to form bisulphite, but as the sulphite present in the liquor is consumed by reaction on the cellulosic material, more bisulphite is formed from the excess sulphate present in the liquor. By 20 injecting the added chemicals in the sulphurous acid solution in the digester, the liquor and chips may be held at a temperature of 250° to 260° F., under which temperature conditions it is desired to effect the treatment 25 with the resulting bisulphite liquor. If the combined  $\text{SO}_2$  content of the liquor is greater than, say, 1% to 2%, the temperature of cooking may be advantageously raised to, say, 285° to 300° F. The treatment with the 30 bisulphite liquor may be for one to two hours, at the end of which time examination of the cellulosic material indicates that it is still in the form of firm chips, even though some softening has taken place. The bisulphite liquor 35 is then withdrawn from the digester and the chips are preferably washed in order to avoid loss of alkali from the alkaline cooking liquor by reaction with free acid carried by the chips. The washed or unwashed chips are then 40 digested in an alkaline liquor the alkalinity of which is afforded by the hydroxide, sulphide, or sulphite of sodium, or by a combination of these chemicals. The alkaline liquor need contain only about one pound of active alkali 45 per cubic foot, calculated as  $\text{Na}_2\text{O}$ , to complete fiber liberation, such an alkalinity being about half that required in the alkaline liquor used for the production of kraft pulp. Preferably, the liquor contains alkali in the 50 form of caustic soda and sodium sulphide, about 40% of this alkali being present as sodium sulphide as in a typical kraft liquor, as such a liquor has been found to yield pulps of the best papermaking characteristics. The 55 time of cooking necessary to effect fiber liberation is much shorter than that required in the kraft process, assuming that cooking is effected under the same temperature and pressure conditions used in the kraft process. Thus, when cooking is effected under the usual 60 temperature and pressure conditions used in the kraft process, say, 300° to 335° F. and 67 to 110 pounds pressure, it is found that complete fiber liberation is effected in about two 65 hours. The resulting pulp, after being

washed free of spent cooking liquor and analyzed, shows an alpha cellulose content of 96% to 98%, a pentosan content of less than 1%, and a viscosity of about 1. Such a product compares favorably with wood pulps 70 which have been refined by subjecting chemical wood pulps such as sulphite or kraft, to chemical refining treatments; and in fact it is of higher alpha cellulose but of lower pentosan content and has a lower solution viscosity. The solution viscosity value of the pulp is considerably lower than that of the usual commercial wood pulps, such as sulphite or kraft, or refined pulps prepared 75 therefrom. The raw pulp obtained by a process such as described may be bleached to whiteness in the usual bleach liquors, but it is preferable to employ a bleach liquor containing sufficient free alkali to maintain a condition of distinct alkalinity in the liquor 80 throughout the bleaching operation, in order to preserve the alpha cellulose content of the pulp while coloring matters are being removed.

The broad principles of the process hereinbefore described may be applied by treating the raw cellulosic material first with the bisulphite liquor and then with the sulphurous acid solution. The bisulphite treatment, if practised under the conditions previously 90 described, will not be accompanied by a substantial isolation of fiber, but the subsequent treatment should be carried out in a sulphurous acid solution containing only about 1% to 2%  $\text{SO}_2$ , in order to avoid substantial fiber 95 liberation. Such a sequence of steps does not, however, permit the use of the first liquor together with its heat and chemicals in the second treatment, as is the case when a sulphurous acid solution is employed in the 100 initial treatment.

It is important that the completion of fiber liberation during the first two treatments be avoided as much as possible in producing the product of the present invention, as the action of an acid solution, particularly of a hot sulphurous acid solution, on a liberated pulp is to injure the pulp seriously for papermaking purposes, as well as to diminish the yield of product obtained after digestion in the alkaline liquor. By permitting the acid solution to act on the cellulosic material while it is associated with non-fibrous organic material on which the acid solution may exert a selective chemical action, the fiber content of the cellulosic material may be preserved to a considerably greater degree.

I claim:

1. A multiple-step process of fiber liberation, in which the fiber content of raw cellulosic material is liberated in the last step, which comprises subjecting the raw cellulosic material to the independent action of a sulphurous acid solution and of a bisulphite solution, and then cooking the material so treated

in an alkaline liquor to complete fiber libera-  
tion.

2. A multiple-step process of fiber libera-  
tion, which comprises cooking raw cellulosic  
5 material successively in a sulphurous acid  
solution, a bisulphite solution, and an alkaline  
liquor, while keeping such material short of  
complete fiber liberation until the alkaline  
liquor exerts its action thereon.
- 10 3. A process of fiber liberation, which com-  
prises cooking raw cellulosic material in a  
sulphurous acid solution, converting the hot  
sulphurous acid solution into a bisulphite liq-  
15 uor, cooking in the bisulphite liquor short  
of fiber liberation, and finally cooking in an  
alkaline liquor to complete fiber liberation.

In testimony whereof I have affixed my sig-  
nature.

GEORGE A. RICHTER.

20

25

30

35

40

45

50

55

60